

J. H. PROCTER.

METHOD OF PRODUCING IRON SHEETS BY ELECTRICAL DEPOSITION.  
APPLICATION FILED SEPT. 7, 1917.

1,300,296.

Patented Apr. 15, 1919.



Fig. 1



Fig. 2



Fig. 3

WITNESSES:

*Felix C. Rodgers.*

*Elmer V. Griggs*

INVENTOR

*Joseph H. Procter*

BY

*Merley G. Carr*

ATTORNEY

# UNITED STATES PATENT OFFICE.

JOSEPH H. PROCTER, OF WILKINSBURG, PENNSYLVANIA, ASSIGNOR TO WESTINGHOUSE ELECTRIC & MANUFACTURING COMPANY, A CORPORATION OF PENNSYLVANIA.

## METHOD OF PRODUCING IRON SHEETS BY ELECTRICAL DEPOSITION.

1,300,296.

Specification of Letters Patent. Patented Apr. 15, 1919.

Application filed September 7, 1917. Serial No. 190,113.

To all whom it may concern:

Be it known that I, JOSEPH H. PROCTER, a citizen of the United States, and a resident of Wilkinsburg, in the county of Allegheny and State of Pennsylvania, have invented a new and useful Improvement in Methods of Producing Iron Sheets by Electrical Deposition, of which the following is a specification.

My invention relates to a method of producing iron sheets by electrical deposition, and it has for an object to provide a method of production of iron laminæ or sheets that may be readily separated from the electrodes upon which they are deposited and hence be cheaply and easily manufactured.

Another object of my invention is to enable the production of very thin plates or thick sheets without distorting or straining them.

A further object of my invention is to produce, in a simple manner, a plate consisting of a series of laminæ that may be machined or punched into field-pole structures.

A still further object of my invention is to produce a structure composed of a plurality of laminæ that may be stamped or otherwise worked as a single unit and then separated into individual laminæ, with a minimum expense.

It is well known that iron sheets for electrical devices could be cheaply constructed by the electrical deposition method if it were not for the fact that the deposited iron must be stripped from the electrode. According to my invention, an electrode is covered, by electro-deposition, with iron to the thickness of a single lamination and then coated with some substance, preferably such as an oxid, that will not be affected by annealing. A coat of graphite is then applied and another layer of iron electrolytically deposited, this process continuing until the desired number of electro-depositions has been obtained.

In the drawing accompanying the specification, Figure 1 is a section of a structure produced according to my invention; Fig. 2 is a vertical section of a conventional cell for depositing iron; and Fig. 3 is a section of a modified form of cell.

Referring to Fig. 1, member 1 is an electrode upon which an iron lamination 2 has been electrically deposited. A coating 3 of soluble material may be painted or burnished upon the deposited lamination 2. This coating 3 is, in turn, coated with a layer 4 of

graphite or other conducting material, upon which an iron lamination 5 may be electrolytically deposited.

In Fig. 2 is shown a container 6 for the electrolyte having electrodes 7 and 8. Electrode 7, upon which the iron is to be deposited, has a cap member 9, preferably detachably connected thereto, the cap member 9 being provided with a supporting member 10. Electrode 7 may be of any desired form but preferably of plate-shape. The electric current is passed from electrode 8 through the electrolyte, during the first operation of the device, to the electrode 7 and then through cap 9 and support 10 in series. After the first lamination is deposited, the electrode 7 is removed from the electrode and coated successively with oxid and graphite. In the next operation, the electrode is replaced in the cell and current is passed from electrode 8 through the electrolyte to the graphite coating and thence to cap member 9. In each instance, the exposed surface of cap member 9 is covered with wax or other similar material and a strip of this on the lower face of cap 9 adjacent electrode 7 is removed to enable the graphite to make electrical contact with cap member 9. The wax coating prevents deposition of metal upon the cap member.

In Fig. 3, a cylindrical electrode 11, corresponding to electrode 7 in Fig. 2, is shown with a circular cap member 12 and a supporting member 13. Surrounding electrode 11, and preferably concentric with it, is an annular electrode 14. A container 15 is provided for the electrolyte. The operation of this modified form of my invention is, in all respects, similar to that of the form illustrated in Fig. 2 and hence need not be set forth in detail.

The method of my invention produces a laminated structure that may be worked or machined into field pole pieces or various other desired forms.

Where it is desirable to anneal the laminated structure, the oxid or non-conducting coating should be of material not affected by the annealing process.

In many instances, it is desirable to have interlaced plates. In such cases, the material with which the successive metal laminæ are coated must be of such nature that it may be dissolved or liquefied without destroying the metal laminæ. Under certain

conditions, a ferrous oxid may be used and dissolved out by sulfuric acid, which, at certain concentration, will have little effect upon the deposited iron. Numerous other 5 equivalent non-conducting coating substances will suggest themselves to one skilled in this art.

In some cases, a wax, which may be readily melted, may be used to coat the deposited 10 iron where it is desired to separate the iron sheets or laminae.

Obviously, other forms of electrodes and conducting materials may be used.

While I have herein shown and described 15 different embodiments of apparatus for carrying out my invention, it will be understood that various modifications may be effected by anyone skilled in the art without departing from the spirit of my invention. 20

I claim as my invention:

1. A method of building up composite structures which consists in electro-depositing a metallic layer, covering said metallic 25 layer with a substantially non-conducting

material to insulate it, coating said non-conducting material with graphite, and electro-depositing a second metallic layer upon said coating of graphite.

2. A method of producing metallic sheets 30 which consists in forming superposed sheets by electro-deposition and coating, in succession, and finally dissolving the intermediate sheets of coating material to separate the electro-deposited sheets. 35

3. A coherent composite structure consisting of alternate layers of electro-deposited metal, an oxid and non-metallic material.

4. A method of building up laminated metallic structures which comprises forming a 40 metallic sheet by electro-deposition, providing an oxid coating thereon, applying a non-metallic current-conducting coating thereto and electrolytically depositing a second metallic sheet upon the latter coating. 45

In testimony whereof, I have hereunto subscribed my name this 31st day of August, 1917.

JOSEPH H. PROCTER.